

## 1

3,111,466

## ELECTRODEPOSITION OF NICKEL

Donald Gardner Foulke, Watchung, William B. Stoddard, Jr., Matawan, Otto Kardos, Red Bank, and Walter B. Kleiner, Plainfield, N.J., assignors to Hanson-Van Winkle-Munning Company, a corporation of New Jersey

No Drawing. Filed Mar. 11, 1959, Ser. No. 798,583  
12 Claims. (Cl. 204—49)

This invention relates to electroplating and, more particularly, to electrodepositing nickel from an aqueous acidic nickel plating bath. The invention is based on the discovery that certain 1,2-benzopyrones, when incorporated in a nickel plating bath in conjunction with various water-

## 2

benzopyrone compound in the bath should be maintained at or near its saturation point.

Any 1,2-benzopyrone compound which is capable of being dissolved by acid and which does not undergo decomposition upon protonation may be selected for inclusion in the plating solution, provided the compound is not sterically hindered nor impeded in its approach to the cathode. The compounds listed in Table I are examples of 1,2-benzopyrones which have been used successfully in plating baths containing various water-soluble acetylenic brighteners. These 1,2-benzopyrone compounds, including coumarin and substituted coumarins, may be used over a very wide range of concentrations, but they are preferably employed in an amount in the range from 25 milligrams per liter to a saturation concentration.

TABLE I

## 1,2-Benzopyrone Compounds



| Compound             | R <sub>a</sub>      | R <sub>b</sub>   | R <sub>c</sub> | R <sub>d</sub> | R <sub>e</sub>      | R <sub>f</sub>   |
|----------------------|---------------------|------------------|----------------|----------------|---------------------|------------------|
| Coumarin             | —H                  | —H               | —H             | —H             | —H                  | —H               |
| 3-Bromocoumarin      | —Br                 | —H               | —H             | —H             | —H                  | —H               |
| 3-Chlorocoumarin     | —Cl                 | —H               | —H             | —H             | —H                  | —H               |
| 3-Acetylcoumarin     | —OCOCH <sub>3</sub> | —H               | —H             | —H             | —H                  | —H               |
| 4-Methylcoumarin     | —H                  | —CH <sub>3</sub> | —H             | —H             | —H                  | —H               |
| 4,8-Dimethylcoumarin | —H                  | —CH <sub>3</sub> | —H             | —H             | —H                  | —CH <sub>3</sub> |
| 6-Methylcoumarin     | —H                  | —H               | —H             | —H             | —CH <sub>3</sub>    | —H               |
| 7-Methoxycoumarin    | —H                  | —H               | —H             | —H             | —OCOCH <sub>3</sub> | —H               |

soluble acetylenic brightening addition agents, are remarkably effective for promoting the formation of ductile electroplates which are much smoother than the base metal plated in such a bath. This ability of an electroplating bath to improve on the smoothness of the basis metal is known as leveling ability and can be used industrially to reduce or eliminate mechanical or electrochemical finishing of the base metal.

We have found that in all instances the combined use of a 1,2-benzopyrone compound and a water-soluble acetylenic compound exerts a synergistic effect on the leveling capacity of the bath as compared with the use of either compound alone. In addition to being notably smoother than the base metal, electrodeposits of nickel formed from a plating bath containing both a 1,2-benzopyrone and an acetylenic brightening addition agent have also been found to be exceptionally resistant to corrosion, even when the electroplate is subjected to the most severe accelerated corrosion tests.

Only relatively small quantities of these 1,2-benzopyrone compounds are required in the plating bath when they are used in conjunction with a water-soluble acetylenic compound, for, in general, concentrations as low as 25 milligrams per liter have been found to promote effective leveling. In many cases, however, at least 50 milligrams per liter of the 1,2-benzopyrone compound should be employed to secure a high leveling effect in the bath. To obtain maximum leveling, the concentration of the 1,2-

Coumarin or a substituted coumarin is employed in the plating bath in conjunction with a water-soluble acetylenic compound, particularly the oxygen-containing acetylenic compounds. Plating baths which contain coumarin (or a substituted coumarin) together with a water-soluble acetylenic brightener additive have a much wider brightening capacity and more often yield bright and ductile electrodeposits than baths which contain either additive alone. Our experiments indicate that any water-soluble acetylenic compound effectively cooperates to some degree with the 1,2-benzopyrone compound for enhancing the leveling, uniformity of brightness, and ductility of the nickel electroplate, though some acetylenic compounds are more effective than others.

The common structural feature of these water-soluble acetylenic compounds is the presence of a highly nucleophilic triple bond which is neither sterically hindered nor impeded in approaching the cathode. Only relatively small quantities of the acetylenic compounds are required in the plating bath when used in conjunction with a 1,2-benzopyrone compound. Concentrations as low as 0.1 millimole per liter, or even less, are effective in some cases, though in general it is preferable to employ at least 1 millimole per liter. There appears to be no critical upper limit on the concentration of these acetylenic brighteners save solubility, but there is no advantage generally in employing more than 25 millimoles per liter, and in most

plating baths substantially the full benefit of their presence is achieved with concentrations in the range from 1 to 10 millimoles per liter.

A preferred process according to this invention for producing a ductile, corrosion-resistant nickel deposit substantially smoother than the basis metal to which it is applied comprises electrodepositing nickel from an aqueous acidic solution of at least one nickel salt in which there is dissolved (a) from about 25 milligrams per liter to a saturation concentration of a 1,2-benzopyrone compound of the group consisting of coumarin and substituted coumarins in which at least one of the hydrogen atoms is replaced with a substituent selected from the group consisting of alkyl radicals, alkoxy radicals, acyl radicals, and halogen radicals, and (b) from 0.1 to 10 millimoles per liter of a water-soluble acetylenic compound.

While any water-soluble acetylenic compound may be employed in the plating bath conjointly with coumarin or a substituted coumarin to produce corrosion-resistant and ductile nickel deposits in accordance with the invention, particularly satisfactory results have been obtained using  $\alpha$ -substituted acetylenic compounds having a structure represented by the formula



and alkynyl groups,  $R_3$  is a substituent of the group consisting of hydrogen, halogen, alkyl, alkenyl, alkynyl, hydroxy-substituted and alkoxy-substituted alkenyl and alkynyl groups, and substituted-alkyl groups having the structural configuration



- 10 in which each of  $R_4$  and  $R_5$  are substituents of the group consisting of hydrogen, alkyl, alkenyl, alkynyl, and hydroxy-substituted and alkoxy-substituted alkyl, alkenyl, and alkynyl groups, and each of  $R_a$  and  $R_a'$  are substituents of the group consisting of hydroxy, alkoxy, carboxy-substituted alkoxy, formoxy, alkanoxy, halogen, and polyoxy groups. Where  $R_3$  is a substituted-alkyl group having the above-illustrated structural configuration, then the acetylenic compound is termed an  $\alpha,\alpha'$ -disubstituted acetylenic compound, since both carbon atoms vicinal to the same acetylenic bond contain either the same or a different functional group. The compounds listed in Table II are examples of various  $\alpha$ -substituted acetylenic compounds which may be used successfully in plating baths containing coumarin or a substituted coumarin. As indicated previously, these acetylenic compounds are preferably used in concentrations from about 1 to about 10 millimoles per liter.

TABLE II  
 $\alpha$ -Substituted Acetylenic Compounds



| Compound                                                               | $R_1$              | $R_2$   | $R_3$                                    | $R_a$                                     |
|------------------------------------------------------------------------|--------------------|---------|------------------------------------------|-------------------------------------------|
| 3-Butyne-1,2-diol.....                                                 | $-CH_2OH$          | $-H$    | $-H$                                     | $-OH$                                     |
| 3-Methyl-1-butyne-3-ol.....                                            | $-CH_3$            | $-CH_3$ | $-H$                                     | $-OH$                                     |
| 3-Methyl-1-pentyne-3-ol.....                                           | $-C_2H_5$          | $-CH_3$ | $-H$                                     | $-OH$                                     |
| 2-Propyn-1-ol.....                                                     | $-H$               | $-H$    | $-H$                                     | $-OH$                                     |
| 2,5-Dimethyl-1-octen-3-yn-5-ol.....                                    | $-C_3H_7$          | $-CH_3$ | $CH_3$<br>$\quad\quad\quad-C\equiv CH_2$ | $-OH$                                     |
| 3-Methyl-1-nonyn-3-ol.....                                             | $-C_6H_{13}$       | $-CH_3$ | $-H$                                     | $-OH$                                     |
| 2,4-Hexadiyne-1,6-diol.....                                            | $-H$               | $-H$    | $\equiv C-C-CH_2OH$                      | $-OH$                                     |
| 1-Methoxy-2-propyne.....                                               | $-H$               | $-H$    | $\equiv C-CH$                            | $-OCH_3$                                  |
| 3-Methoxy-3-methyl-4,6-heptadiyne.....                                 | $-C_2H_5$          | $-CH_3$ | $\equiv C-CH$                            | $-OCH_3$                                  |
| 3-Ethoxy-3,5,7-trimethyl-1-octyne.....                                 | $-C_7H_{15}$       | $-CH_3$ | $-H$                                     | $-OCH_3$                                  |
| 1-Formoxy-2-propyne.....                                               | $-H$               | $-H$    | $-H$                                     | $-OCH_2$                                  |
| 1-Acetoxy-2-propyne.....                                               | $-H$               | $-H$    | $-H$                                     | $-OCC_2H_5$                               |
| 3-Methyl-1-nonyn-3-yl acetate.....                                     | $-C_6H_{13}$       | $-CH_3$ | $-H$                                     | $-OCC_2H_5$                               |
| 3-Methyl-1-butyn-3-yl acetate.....                                     | $-CH_3$            | $-CH_3$ | $-H$                                     | $-OCC_2H_5$                               |
| 1-Chloro-6-methoxy-2,4-hexadiyne.....                                  | $-H$               | $-H$    | $\equiv C-C-CH_2OCH_3$                   | $-Cl$                                     |
| 3-Chloro-3-methyl-4-hexyne.....                                        | $-C_2H_5$          | $-CH_3$ | $\equiv C-CH_3$                          | $-Cl$                                     |
| 1-Bromo-2-propyne.....                                                 | $-H$               | $-H$    | $\equiv C-CH_3$                          | $-Br$                                     |
| 1,2-Di-( $\beta$ -hydroxyethoxy)-3-butyne.....                         | $-CH_2OCH_2CH_2OH$ | $-H$    | $\equiv C-CH_3$                          | $-OCH_2CH_2OH$                            |
| 3-( $\beta$ -Hydroxy- $\gamma$ -chloropropoxy)-3-methyl-4-pentyne..... | $-C_2H_5$          | $-CH_3$ | $-H$                                     | $CH_2Cl$<br>$\quad\quad\quad-OCH_2CH_2OH$ |
| 3-( $\beta$ , $\gamma$ -Epoxypropoxy)-3-methyl-4-pentyne.....          | $-C_2H_5$          | $-CH_3$ | $-H$                                     | $O$<br>$\quad\quad\quad-OCH_2CH_2CH_2O$   |

in which each of  $R_1$  and  $R_2$  are substituents of the group consisting of hydrogen, alkyl, alkenyl, alkynyl, and hydroxy-substituted and alkoxy-substituted alkyl, alkenyl, 75

Table III sets forth examples of  $\alpha,\alpha'$ -disubstituted acetylenic compounds which, when used in the plating bath in conjunction with a 1,2-benzopyrone compound, yield

nickel electroplates which are exceptionally resistant to corrosion and possess improved ductility.

polyethoxy)-2-butyne has been found to be exceptionally pronounced when the bath is operated at temperatures

TABLE III  
*α,α'-Disubstituted Acetylenic Compounds*

| Compound                                                 | R <sub>1</sub>                 | R <sub>2</sub>   | R <sub>4</sub>                 | R <sub>5</sub>                 | R <sub>α</sub>                               | R <sub>α'</sub>                              |
|----------------------------------------------------------|--------------------------------|------------------|--------------------------------|--------------------------------|----------------------------------------------|----------------------------------------------|
| 2-Butyne-1,4-diol                                        | —H                             | —H               | —H                             | —H                             | —OH                                          | —OH                                          |
| 2,5-Dimethyl-3-hexyne-2,5-diol                           | —CH <sub>3</sub>               | —CH <sub>3</sub> | —CH <sub>3</sub>               | —CH <sub>3</sub>               | —OH                                          | —OH                                          |
| 4,7-Dimethyl-5-decyn-4,7-diol                            | —C <sub>3</sub> H <sub>7</sub> | —CH <sub>3</sub> | —CH <sub>3</sub>               | —C <sub>3</sub> H <sub>7</sub> | —OH                                          | —OH                                          |
| 3,6-Dimethyl-1,7-octadien-4-yne-3,6-diol                 | —C <sub>2</sub> H <sub>5</sub> | —CH <sub>3</sub> | —C <sub>2</sub> H <sub>5</sub> | —C <sub>2</sub> H <sub>5</sub> | —OH                                          | —OH                                          |
| 2,5-Diphenyl-3-hexyne-2,5-diol                           | —C <sub>6</sub> H <sub>5</sub> | —CH <sub>3</sub> | —CH <sub>3</sub>               | —C <sub>6</sub> H <sub>5</sub> | —OH                                          | —OH                                          |
| 4-Methoxy-2-buty-1-ol                                    | —H                             | —H               | —H                             | —H                             | —OCH <sub>2</sub> CH <sub>2</sub> OH         | —OCH <sub>2</sub> CH <sub>2</sub> OH         |
| 1,4-Di-(β-hydroxyethoxy)-2-butyne                        | —H                             | —H               | —H                             | —C <sub>3</sub> H <sub>7</sub> | —OCH <sub>2</sub> CH <sub>2</sub> OH         | —OCH <sub>2</sub> CH <sub>2</sub> OH         |
| 4,7-Di-(β-hydroxy-γ-chloropropoxy)-4,7-dimethyl-5-decyne | —C <sub>3</sub> H <sub>7</sub> | —CH <sub>3</sub> | —CH <sub>3</sub>               | —C <sub>3</sub> H <sub>7</sub> | —OCH <sub>2</sub> CH <sub>2</sub> OH         | —OCH <sub>2</sub> CH <sub>2</sub> OH         |
| 1,4-Di-(β-hydroxy-γ-chloropropoxy)-2-butyne              | —H                             | —H               | —H                             | —H                             | CH <sub>2</sub> Cl<br>—OCH <sub>2</sub> CHOH | CH <sub>2</sub> Cl<br>—OCH <sub>2</sub> CHOH |
| 3,6-Di-(β-hydroxy-γ-chloropropoxy)-1,4,7-octatriyne      | —C≡CII                         | —H               | —H                             | —C≡CII                         | CH <sub>2</sub> Cl<br>—OCH <sub>2</sub> CHOH | CH <sub>2</sub> Cl<br>—OCH <sub>2</sub> CHOH |
| 1,4-Diacetoxy-2-butyne                                   | —H                             | —H               | —H                             | —H                             | —O—C(=O)CH <sub>3</sub>                      | —O—C(=O)CH <sub>3</sub>                      |
| 1,4-Dichloro-2-butyne                                    | —H                             | —H               | —H                             | —H                             | —Cl                                          | —Cl                                          |
| 4-Chloro-2-buty-1-ol                                     | —H                             | —H               | —H                             | —H                             | —Cl                                          | —OH                                          |
| 3,6-Dimethoxy-1,4,7-octatriyne                           | —C≡CII                         | —H               | —H                             | —C≡CII                         | —OCH <sub>3</sub>                            | —OCH <sub>3</sub>                            |

Among the most satisfactory acetylenic brightening agents are those prepared by reacting either an α-hydroxy or an α,α'-dihydroxy acetylenic compound, such as those listed in Tables II and III, with either ethylene oxide or epichlorohydrin. These adducts readily dissolve in acidic nickel plating baths, and are unusually effective in such baths both in promoting the formation of bright and ductile electrodeposits over wide current density ranges and in exerting a pronounced leveling effect on the bath during the plating operation. Two such adducts which are notably effective when used in conjunction with the 1,2-benzopyrone compound, particularly with 3-bromocoumarin, are the α,α'-di-(polyoxy)-2-butyne obtained upon the reaction of 2-butyne-1,4-diol with ethylene oxide and with epichlorohydrin.

2-butyne-1,4-diol reacts with ethylene oxide in the presence of a base to form a 1,4-di-(hydroxypolyethoxy)-2-butyne which is structurally characterized by the formula



and with epichlorohydrin to form a 1,4-di-[hydroxypoly(β-chloromethylethoxy)]-2-butyne, the structure of which is represented by the formula



*n* in both formulas being an integer from 1 to 20. The leveling effect of both of these reaction products in combination with coumarin or various substituted coumarins in nickel plating baths is especially pronounced.

Outstanding results have been obtained when these water-soluble acetylenic compounds are used in the bath in conjunction with 3-bromocoumarin, the structure of which is represented by the following formula:



The leveling effect of 3-bromocoumarin used in conjunction with either 2-butyne-1,4-diol or a 1,4-di-(hydroxy-

ranging from about 50° C. to about 85° C. and at a pH from about 3.0 to 4.5 and when the concentration of 3-bromocoumarin is maintained at or near its saturation point. To maintain the concentration of 3-bromocoumarin at this optimum level in the plating bath, the electrolyte may be circulated continuously through a filter pad consisting of diatomaceous earth mixed with crystalline 3-bromocoumarin. By using this method, it is impossible to supersaturate the plating solution with the bromocoumarin compound no matter at which temperature the bath is operated since the maximum solubility of 3-bromocoumarin in the electrolyte is that at which substantially maximum leveling is obtained. Moreover, the melting point of 3-bromocoumarin is appreciably higher than the highest temperatures used in most commercial bright nickel plating processes, and consequently there is no objectionable introduction of molten compound into the bath even at the maximum commercial plating temperatures. By using 3-bromocoumarin in the plating solution, it is possible to employ both higher temperatures and higher current densities and to complete the plating operation more rapidly than can be done by using any other 1,2-benzopyrone compound in the bath.

The following examples, which are summarized in Tables IV through VI, are illustrative of the effectiveness with which coumarin and substituted coumarins may be used in conjunction with various water-soluble acetylenic brightening addition agents in accordance with this invention. In each example, the electrodeposit was formed from a Watts plating bath having the following basic composition:

|                                                            | Grams per liter |
|------------------------------------------------------------|-----------------|
| Nickel sulfate, $\text{NiSO}_4 \cdot 7\text{H}_2\text{O}$  | 300             |
| Nickel chloride, $\text{NiCl}_2 \cdot 6\text{H}_2\text{O}$ | 45              |
| Boric acid, $\text{H}_3\text{BO}_3$                        | 41.25           |

Plating operations in each example were carried out in an open vessel on steel and polished stainless steel cathodes, using vigorous air agitation, a bath pH of about 4.0, a bath temperature of 60° C., and an average current density of 60 amperes per square foot. The average thickness of each electrodeposit was 0.025 millimeter (0.001 inch).

Table IV sets forth the results obtained when nickel was electrodeposited from the standard Watts plating bath which contained varying concentrations of 3-bromocoumarin, alone and in combination with a representative water-soluble acetylenic compound. In each of the examples summarized in Table IV, the foil ductility of the plated panel was determined by the Chrysler foil ductility test (in which the foil is removed from the plated panel and then bent between the jaws of a micrometer until it cracks, foil ductility being defined as the ratio of the foil thickness to the micrometer reading when cracking first occurs), the theoretically maximum value being 0.5 for brittle nickel electrodeposits. The leveling effect exerted by the bath, which is a measure of the decrease in roughness of the nickel electrodeposit compared to that of the underlying metal surface, was also determined in each of these examples by measuring the surface roughness (root mean square value in microinches) of the steel panel with a brush surface analyzer prior to the plating operation and then immediately following the plating operation.

TABLE IV

*Cumulative Effect of 3-Bromocoumarin and Various Acetylenic Compounds on the Leveling and Ductility of Nickel Electrodeposits*

| Acetylenic Compound                            | Conc., gm./l. | 3-Bromo-<br>cou-<br>marin,<br>mg./l. | Character of<br>Electrodeposit |           |               |
|------------------------------------------------|---------------|--------------------------------------|--------------------------------|-----------|---------------|
|                                                |               |                                      | Leveling,<br>percent           | Ductility | D-L<br>Factor |
| None.....                                      | 0.0           | 80                                   | 88                             | 0.5       | 34.0          |
| 2-Butyne-1,4-diol.....                         | 0.10          | 0.0                                  | 50.6                           | 0.0       | 0.0           |
|                                                | 0.10          | 80                                   | 75                             | 0.5       | 37.5          |
|                                                | 0.10          | 123                                  | 83                             | 0.5       | 41.5          |
|                                                | 0.112         | 58                                   | 71.9                           | 0.5       | 35.95         |
| 3-Methyl-1-butyne-3-ol.....                    | 0.05          | 80                                   | 73                             | 0.5       | 36.5          |
| 1-Bromo-2-propyne.....                         | 0.05          | 80                                   | 77.5                           | 0.5       | 38.75         |
| 1,4-Di-( $\beta$ -hydroxyethoxy)-2-butyne..... | 0.106         | 80                                   | 75                             | 0.5       | 37.5          |
| 3-Methyl-3-buten-1-yne.....                    | 0.090         | 80                                   | 70                             | 0.5       | 35.0          |
| 1,4-Dichloro-2-butyne.....                     | 0.15          | 100                                  | 82                             | 0.5       | 41.0          |
| Propiolic acid.....                            | 0.20          | 80                                   | 81                             | 0.5       | 40.5          |

Table V summarizes the results of a series of tests which demonstrate the effectiveness of coumarin in improving both the foil ductility as well as the adhesion to the basis metal of deposits produced from baths containing various acetylenic compounds without substantially diminishing the pronounced characteristic leveling effect exerted on plating solutions by acetylenic compounds. The pH of the bath was adjusted to about 4.5 in each case, and the electrodeposit formed at a temperature of 60° C., using mild air agitation and an average current density of 60 amperes per square foot.

TABLE V

*Effect of Coumarin and Various Acetylenic Compounds on the Ductility and Leveling of Nickel Electrodeposits*

| Acetylenic Compound                            | Conc., gm./l. | Cou-<br>marin,<br>mg./l. | Character of<br>Electrodeposit |           |               |
|------------------------------------------------|---------------|--------------------------|--------------------------------|-----------|---------------|
|                                                |               |                          | Leveling,<br>percent           | Ductility | D-L<br>Factor |
| None.....                                      | 0.0           | 50                       | 60                             | 0.5       | 30.0          |
| 2-Butyne-1,4-diol.....                         | 0.1           | 0.0                      | 50.0                           | 0         | 0             |
|                                                | 0.15          | 80                       | 86.5                           | 0.5       | 43.25         |
| 1,4-Di-( $\beta$ -hydroxyethoxy)-2-butyne..... | 0.1           | 0.0                      | 40                             | 0.5       | 20.0          |
|                                                | 0.15          | 50                       | 70                             | 0.5       | 35.0          |
| 1-Bromo-2-propyne.....                         | 0.15          | 50                       | 65                             | 0.5       | 32.5          |
| 1,4-Dichloro-2-butyne.....                     | 0.05          | 50                       | 65                             | 0.5       | 32.5          |

The general principle illustrated in Tables IV and V, that coumarin or substituted coumarins are capable of functioning as "carrier" brighteners when used in a nickel plating bath in conjunction with a water-soluble acetylenic brightener, was repeatedly and consistently verified in another series of tests using a variety of acetylenic

70 75

brighteners, including many representative alkynol-epoxide adducts. Although the basis or reaction mechanism by which these 1,2-benzopyrone compounds function in a nickel plating bath in combination with acetylenic brighteners is not completely understood, it is apparent from the examples summarized in Tables IV and V that the plating bath must contain both the 1,2-benzopyrone compound and the acetylenic brightener to obtain both the maximum ductility together with leveling, the criterion of which is indicated by a high D-L factor which, in turn, is defined as the product of the foil ductility times the leveling. Moreover, electrodeposition of nickel formed from a bath containing both the 1,2-benzopyrone compound and an acetylenic brightener possess an exceptionally notable resistance to corrosion, even when subjected to the most severe accelerated corrosion tests.

To illustrate the improved corrosion resistance exhibited by electrodeposits formed from plating baths containing a 1,2-benzopyrone compound and a water-soluble acetylenic brightener in accordance with the invention, Table VI lists the corrosion ratings of four duplex-plated panels produced from the basic Watts plating bath which contained an acetylenic compound together with either a 1,2-benzopyrone compound (3-bromocoumarin or coumarin) or a sulfo-oxygen "carrier" addition agent (sodium naphthalene-1,3,6-trisulfonate). As before, plating operations were carried out in an open vessel on steel panels, using substantially the same conditions as previously described, each panel receiving a duplex coating having an average thickness of 1.5 mils. Each of the plated panels was coated with a synthetic soil consisting of a paste prepared by dispersing 0.035 gram of cupric nitrate, 0.165 gram of ferric chloride, 1.0 gram of ammonium chloride, and 30.0 grams of kaolin in 50.0 milliliters of distilled water. After each panel had been uniformly coated with a layer of the synthetic soil, the coated panel was exposed to a constant humidity of about 90 percent at a temperature of 100° F. for a period of 24 hours, following which the synthetic soil was removed by washing and the panel then immersed in boiling water for an additional 24 hours. The relative corrosion resistance of each electroplate is expressed in terms of its Corrodekote rating which was determined by the official Corrodekote Test of the American Electroplaters' Society. This rating is graded on a logarithmic scale from zero (negligible corrosion resistance) to 10 (complete corrosion resistance), values above 9.0 representing exceptionally high resistance to corrosion.

TABLE VI  
*Relative Corrosion Resistance of Nickel Electrodeposits*

|    | A. Bath Additives:                                   | Bath 1                     | Bath 2 | Bath 3 | Bath 4 |
|----|------------------------------------------------------|----------------------------|--------|--------|--------|
|    |                                                      | 2-Butyne-1,4-diol (gm./l.) | 0.25   | 0.4    | -----  |
| 60 | 1,4-Di-( $\beta$ -hydroxyethoxy)-2-butyne (gm./l.)   | -----                      | -----  | 0.6    | -----  |
|    | Coumarin (mg./l.)                                    | -----                      | 50.0   | -----  | -----  |
|    | 3-Bromocoumarin (mg./l.)                             | -----                      | -----  | 80.0   | -----  |
|    | Sodium naphthalene-1,3,6-trisulfonate (gm./l.)       | -----                      | -----  | -----  | 15.0   |
|    | B. Corrodekote Rating of Electrodeposit (Scale=0-10) | 9.8                        | 9.7    | 9.7    | 6.5    |

65 In the foregoing examples of the invention, coumarin and substituted coumarins in which at least one of the hydrogen atoms is replaced by an alkyl, acyl, alkoxy, or halogen radical were successfully employed in combination with various water-soluble acetylenic compounds in the standard Watts nickel electroplating bath, which is prepared by dissolving nickel sulfate, nickel chloride, and boric acid in water. Similar advantages are also attained when coumarin or substituted coumarins are used in conjunction with the acetylenic brightener additives in other types of aqueous acidic nickel electroplating

baths. For example, these 1,2-benzopyrone compounds are beneficial when used in straight nickel sulfate baths, in nickel sulfate-chloride baths, and in various other nickel plating baths based on using nickel sulfamate or nickel fluoborate as the nickel salt which is dissolved in an aqueous acidic solvent, and consequently the invention is applicable to electroplating from any aqueous acidic solution of one or more nickel salts.

We claim:

1. A process for producing a corrosion-resistant nickel deposit substantially smoother than the basis metal to which it is applied which comprises electrodepositing nickel from an aqueous acidic solution of at least one nickel salt in which there is dissolved (a) from about 25 milligrams per liter to a saturation concentration of a 1,2-benzopyrone compound of the group consisting of coumarin and substituted coumarins in which at least one of the hydrogen atoms is replaced with a substituent selected from the group consisting of alkyl radicals, alkoxy radicals, acyl radicals, and halogen radicals, and (b) from 0.1 to 10 millimoles per liter of a watersoluble acetylenic compound.

2. A process for producing a corrosion-resistant nickel deposit substantially smoother than the basis metal to which it is applied which comprises electrodepositing nickel from an aqueous acidic solution of at least one nickel salt in which there is dissolved (a) from about 25 milligrams per liter to a saturation concentration of a 1,2-benzopyrone compound of the group consisting of coumarin and substituted coumarins in which at least one of the hydrogen atoms is replaced with a substituent selected from the group consisting of alkyl radicals, alkoxy radicals, acyl radicals, and halogen radicals, and (b) from 0.1 to 10 millimoles per liter of an  $\alpha$ -substituted acetylenic compound having a structure represented by the formula



in which each of  $R_1$  and  $R_2$  are substituents of the group consisting of hydrogen, alkyl, alkenyl, alkynyl, and hydroxy-substituted and alkoxy-substituted alkyl, alkenyl, and alkynyl groups,  $R_3$  is a substituent of the group consisting of hydrogen, halogen, alkyl, alkenyl, alkynyl, hydroxy-substituted and alkoxy-substituted alkenyl and alkynyl groups, and substituted-alkyl groups having the structural configuration



in which each of  $R_4$  and  $R_5$  are substituents of the group consisting of hydrogen, alkyl, alkenyl, alkynyl, and hydroxy-substituted and alkoxy-substituted alkyl, alkenyl, and alkynyl groups, and each  $R_a$  and  $R_a'$  are substituents of the group consisting of hydroxy, alkoxy, carboxy-substituted alkoxy, formoxy, alkanoxy, halogen, and polyoxy groups.

3. A process for producing a corrosion-resistant nickel deposit substantially smoother than the basis metal to which it is applied which comprises electrodepositing nickel from an aqueous acidic solution of at least one nickel salt in which there is dissolved (a) from about 25 milligrams per liter to a saturation concentration of a 1,2-benzopyrone compound of the group consisting of coumarin and substituted coumarins in which at least one of the hydrogen atoms is replaced with a substituent selected from the group consisting of alkyl radicals, alkoxy radicals, acyl radicals, and halogen radicals, and (b) from 0.1 to 10 millimoles per liter of an  $\alpha,\alpha'$ -disubstituted acetylenic compound having a structure represented by the formula



in which each of  $R_1$ ,  $R_2$ ,  $R_4$ , and  $R_5$  are substituents of the group consisting of hydrogen, alkyl, alkenyl, alkynyl, and hydroxy-substituted and alkoxy-substituted alkyl, alkenyl, and alkynyl groups, and each of  $R_a$  and  $R_a'$  are substituents of the group consisting of hydroxy, alkoxy, carboxy-substituted alkoxy, formoxy, alkanoxy, halogen, and polyoxy groups.

4. A process for producing a corrosion-resistant nickel deposit substantially smoother than the basis metal to which it is applied which comprises electrodepositing nickel from an aqueous acidic solution of at least one nickel salt in which there is dissolved (a) from about 25 milligrams per liter to a saturation concentration of a 1,2-benzopyrone compound of the group consisting of coumarin and substituted coumarins in which at least one of the hydrogen atoms is replaced with a substituent selected from the group consisting of alkyl radicals, alkoxy radicals, acyl radicals, and halogen radicals, and (b) from 1 to 10 millimoles per liter of a water-soluble acetylenic compound selected from the group consisting of 2-propyn-1-ol, 1-bromo-2-propyne, 1,4-dichloro-2-butyne, 2-butyne-1,4-diol, 3-methyl-1-butyn-3-ol,  $\alpha$ -polyoxy acetylenic compounds having a structure represented by the formula



and  $\alpha,\alpha'$ -di(polyoxy) acetylenic compounds having a structure represented by the formula



5. in which each of  $R_1$ ,  $R_2$ ,  $R_4$ , and  $R_5$  are substituents of the group consisting of hydrogen, alkyl, alkenyl, alkynyl, and hydroxy-substituted and alkoxy-substituted alkyl, alkenyl, and alkynyl groups,  $R_3$  is a substituent of the group consisting of hydrogen, halogen, alkyl, alkenyl, alkynyl, hydroxy-substituted and alkoxy-substituted alkenyl and alkynyl groups, and substituted-alkyl groups having the structural configuration



in which  $R_a$  is a substituent of the group consisting of hydroxy, alkoxy, carboxy-substituted alkoxy, formoxy, alkanoxy, halogen, and polyoxy groups, and  $n$  is an integer from 1 to 20.

5. A nickel electroplating bath for producing a corrosion-resistant nickel deposit substantially smoother than the basis metal to which it is applied comprising an aqueous acidic solution of at least one nickel salt in which there is dissolved from about 25 milligrams per liter to a saturation concentration of 3-bromocoumarin, and from 0.1 to 10 millimoles per liter of a water-soluble acetylenic compound.

6. A nickel electroplating bath for producing a corrosion-resistant nickel deposit substantially smoother than the basis metal to which it is applied comprising an aqueous acidic solution of at least one nickel salt in which there is dissolved from about 25 milligrams per liter to a saturation concentration of 3-bromocoumarin, and from 0.1 to 10 millimoles per liter of an  $\alpha$ -substituted acetylenic compound having a structure represented by the formula



70 in which each of  $R_1$  and  $R_2$  are substituents of the group consisting of hydrogen, alkyl, alkenyl, alkynyl, and hydroxy-substituted and alkoxy-substituted alkyl, alkenyl, and alkynyl groups, and  $R_3$  is a substituent of the group consisting of hydrogen, halogen, alkyl, alkenyl, alkynyl,

75 consisting of hydroxy, alkoxy, carboxy-substituted alkoxy, formoxy, alkanoxy, halogen, and polyoxy groups.

11

hydroxy-substituted and alkoxy-substituted alkenyl and alkynyl groups, and substituted-alkyl groups having the structural configuration



in which each of  $R_4$  and  $R_5$  are substituents of the group consisting of hydrogen, alkyl, alkenyl, alkynyl, and hydroxy-substituted and alkoxy-substituted alkyl, alkenyl, and alkynyl groups, and each of  $R_4'$  and  $R_5'$  are substituents of the group consisting of hydroxy, alkoxy, carboxy-substituted alkoxy, formoxy, alkanoxy, halogen, and polyoxy groups.

7. A nickel electroplating bath for producing a corrosion-resistant nickel deposit substantially smoother than the basis metal to which it is applied comprising an aqueous acidic solution of at least one nickel salt in which there is dissolved from about 25 milligrams per liter to a saturation concentration of 3-bromocoumarin, and from 0.1 to 10 millimoles per liter of an  $\alpha,\alpha'$ -disubstituted acetylenic compound having a structure represented by the formula



in which each of  $R_1$ ,  $R_2$ ,  $R_4$ , and  $R_5$  are substituents of the group consisting of hydrogen, alkyl, alkenyl, alkynyl, and hydroxy-substituted and alkoxy-substituted alkyl, alkenyl, and alkynyl groups, and each of  $R_3$  and  $R_6$  are substituents of the group consisting of hydroxy, alkoxy, carboxy-substituted alkoxy, formoxy, alkanoxy, halogen, and polyoxy groups.

8. A nickel electroplating bath for producing a corrosion-resistant nickel deposit substantially smoother than the basis metal to which it is applied comprising an aqueous acidic solution of at least one nickel salt in which there is dissolved from about 25 milligrams per liter to a saturation concentration of 3-bromocoumarin, and from 1 to 10 millimoles per liter of a water-soluble acetylenic compound selected from the group consisting of 2-propyn-1-ol, 1-bromo-2-propyne, 1,4-dichloro-2-butyne, 2-butyne-1,4-diol, 3-methyl-1-butyn-3-ol,  $\alpha$ -polyoxy acetylenic compounds having a structure represented by the formula



and  $\alpha, \alpha'$ -di(polyoxy) acetylenic compounds having a structure represented by the formula



in which each of  $R_1$ ,  $R_2$ ,  $R_4$ , and  $R_5$  are substituents of the group consisting of hydrogen, alkyl, alkenyl, alkynyl, and

12

hydroxy-substituted and alkoxy-substituted alkyl, alkenyl, and alkynyl groups,  $R_3$  is a substituent of the group consisting of hydrogen, halogen, alkyl, alkenyl, alkynyl, hydroxy-substituted and alkoxy-substituted alkenyl and alkynyl groups, and substituted-alkyl groups having the structural configuration



in which  $R_a$  is a substituent of the group consisting of hydroxy, alkoxy, carboxy-substituted alkoxy, formoxy, alkanoxy, halogen, and polyoxy groups, and  $n$  is an integer from 1 to 20.

From 1 to 20.

15 9. A process for producing a corrosion-resistant nickel deposit substantially smoother than the basis metal to which it is applied which comprises electrodepositing nickel from an aqueous acidic solution of at least one nickel salt in which there is dissolved from about 25 milli-  
20 grams per liter to a saturation concentration of 3-bromo-coumarin, and from 0.05 to  $\frac{1}{4}$  gram per liter of 2-butyne-1,4-diol.

10. A process for producing a corrosion-resistant nickel deposit substantially smoother than the basis metal to  
25 which it is applied which comprises electrodepositing nickel from an aqueous acidic solution of at least one nickel salt in which there is dissolved from about 25 milligrams per liter to a saturation concentration of 3-bromocoumarin, and from 1 to 10 millimoles per liter of a water-  
30 soluble  $\alpha, \alpha'$ -di(polyoxy)-2-butyne having a structure represented by the formula



35. in which  $n$  is an integer from 1 to 20.

11. A process for producing a corrosion-resistant nickel deposit substantially smoother than the basis metal to which it is applied which comprises electrodepositing nickel from an aqueous acidic solution of at least one nickel salt at a temperature from about 50° C. to about 85° C. and at a pH between 3.0 and 4.5 and in which there is dissolved from 0.05 to 1 gram per liter of a water-soluble acetylenic compound while maintaining a saturation concentration of 3-bromocoumarin in the solution.

45 12. A process for producing a corrosion-resistant nickel deposit which comprises electrodepositing nickel from an aqueous acidic solution of at least one nickel salt in which there is dissolved from about 0.2 to 3 grams per liter of coumarin, and from about 0.01 to 1.5 grams per liter of

50 a compound selected from the group consisting of acetylenic alcohols, acetylenic esters and acetylenic ethers.

**References Cited** in the file of this patent

UNITED STATES PATENTS

- 55 2,635,076 Du Rose ----- Apr. 14, 1953  
2,712,522 Kardos et al. ----- July 5, 1955

UNITED STATES PATENT OFFICE  
CERTIFICATE OF CORRECTION

Patent No. 3,111,466

November 19, 1963

Donald Gardner Foulke et al.

It is hereby certified that error appears in the above numbered patent requiring correction and that the said Letters Patent should read as corrected below.

Column 2, Table I, column 6, line 8 thereof, for  
" $\text{OCH}_3$ " read --  $\text{OCH}_3$  --; column 10, line 75, for "ankeny1"  
-- aikenyl --.

Signed and sealed this 28th day of April 1964.

(SEAL)

Attest:

ERNEST W. SWIDER

Attesting Officer

EDWARD J. BRENNER

Commissioner of Patents

UNITED STATES PATENT OFFICE  
CERTIFICATE OF CORRECTION

Patent No. 3,111,466

November 19, 1963

Donald Gardner Foulke et al.

It is hereby certified that error appears in the above numbered patent requiring correction and that the said Letters Patent should read as corrected below.

Column 2, Table I, column 6, line 8 thereof, for  
"-OCH" read -- <sup>3</sup>-OCH<sub>3</sub> --; column 10, line 75, for "alkenyl"  
-- alkenyl --.

Signed and sealed this 28th day of April 1964.

(SEAL)

Attest:

ERNEST W. SWIDER

Attesting Officer

EDWARD J. BRENNER

Commissioner of Patents